

# UNITED STATES PATENT OFFICE.

EMMA S. COLEMAN, OF BEATRICE, NEBRASKA.

## COMPOSITION OF MATTER TO BE USED FOR RENDERING PAPER IMPERVIOUS TO AIR AND MOISTURE.

1,158,897.

Specification of Letters Patent.

Patented Nov. 2, 1915.

No Drawing.

Application filed December 28, 1914. Serial No. 879,326.

*To all whom it may concern:*

Be it known that I, EMMA S. COLEMAN, a citizen of the United States, residing at Beatrice, in the county of Gage and State of Nebraska, have invented a new and useful Composition of Matter to be Used for Rendering Paper Impervious to Air and Moisture, as set forth in the ensuing specification.

10 My composition consists of the following ingredients combined in the proportions stated, viz:

Pure grain alcohol ----- 1 part.

Pure olive oil ----- 1 part.

15 Sheet gutta-percha dissolved in chloroform -----  $\frac{1}{2}$  of 1st part.

Sheet gutta-percha is named in preference to the gutta-percha chips as it dissolves more readily than the latter. Olive oil is preferred to some less expensive oils since it is much less liable to become rancid. Carbon-bi-sulfid may be used to dissolve gutta-percha but, owing to its unpleasant 25 odor, chloroform is named. The olive oil

and dissolved gutta-percha, must first be thoroughly mixed by stirring; the alcohol may then be added and all mingled by agitation. The composition obtained may then be applied to each side of the paper, and the 30 paper dried. The oil and gutta-percha fill the pores of the paper. The alcohol aids the other two ingredients to dry in addition to diluting them to a proper consistency. When dry the paper will resist moisture 35 and, if gathered closely together at the edges the air may be excluded. The pliability and fiber of paper treated by the composition described herein will be found to remain intact. 40

I claim:

The herein-described composition of matter consisting of alcohol, olive oil and a solution of gutta-percha, in the proportions stated, and for the purpose of rendering 45 paper impervious to air and moisture.

EMMA S. COLEMAN.

Witnesses:

L. W. COLBY,  
F. W. MESSMORE.